

# UNITED STATES PATENT OFFICE.

HERBERT PASCHKE, OF BEN AVON HEIGHTS, PENNSYLVANIA, ASSIGNOR TO ARM-  
STRONG CORK COMPANY, OF PITTSBURGH, PENNSYLVANIA, A CORPORATION OF  
PENNSYLVANIA.

## METHOD OF MAKING ARTIFICIAL-CORK ARTICLES.

1,131,860.

Specification of Letters Patent. Patented Mar. 16, 1915.

No Drawing.

Application filed January 25, 1913. Serial No. 744,188.

To all whom it may concern:

Be it known that I, HERBERT PASCHKE, a citizen of the United States, residing at Ben Avon Heights, in the county of Allegheny and State of Pennsylvania, have invented a new and useful Improvement in Methods of Making Artificial-Cork Articles, of which the following is a full, clear, and exact description.

10 My invention has relation to artificial cork articles and to the method of manufacturing the same, and is designed to provide an article of this character which shall be tough, elastic, and water-repellent, and in which the binder is of such character that the article will not dry out or become brittle, and which is insoluble in ordinary solvents, the articles produced being adapted to a wide variety of uses.

20 My invention also provides a novel method of manufacturing such articles, which is capable of being carried out in a commercial way at a relatively low cost.

In accordance with my invention, I mix 25 granulated or pulverized cork particles with tung oil (otherwise known as China or Chinese wood oil, Japanese wood oil, etc.) with or without other ingredients, as hereinafter described. I then compress the cork 30 mass, which has been thoroughly mixed with the oil, in molds of the desired shape and subject the molded mass, while in these closed molds, to the action of heat for a prolonged period of time. The effect of this 35 heating operation is to solidify the tung oil which acts as a binder for the cork particles, and thereby produce a shaped body or article of artificial cork which possesses a high degree of elasticity and toughness, together 40 with the other qualities above named. The degree of temperature employed, as well as the extent of the heating period, will depend largely upon the mass of the molded body, the particular purpose for which the 45 article is to be used, and the nature and amount of other ingredients which may be added.

50 The temperature must in all cases be below the point at which charring or other permanent injury of the cork particles would occur. I have obtained excellent results by the use of a temperature of from 212° to 220° F., the treatment extending over a period of from two to three days.

By the above described method, I am able

to produce a highly desirable article in 55 which the tung oil may be the only binder employed. The efficiency of this material as a binder is due largely to the solidification of the oil, and which I attribute, in part, to oxidation, and in part, to polymerization of the oil; but in view of the high degree of toughness which I obtain, I am inclined to believe that the tung oil mixes or fuses with some of the natural glycerids or fatty acids of the cork. I am 65 strengthened in this belief by the fact that some of these glycerids or fatty acids, which I have been able to isolate, will mix or fuse with the tung oil under the conditions of treatment above described.

70 Other essential or aromatic oils, such as pine oil or turpentine, may be mixed with the tung oil in varying proportions, if desired. The elasticity may be further increased by the addition of rubber dissolved 75 in turpentine. I may also add relatively small quantities of another fatty oil or oils, such as corn oil, poppy seed oil, etc. I may also add different solvents, such as turpentine, benzin, carbon-bisulfid, carbon-tetrachlorid, etc., to facilitate the better distribution 80 of the tung oil in the mass. The natural odor of the tung oil may be overcome or changed by the addition of balsams, resins or other suitable agents. Various coloring 85 matters may also be added to give the formed articles any desired tint or color.

While the amount of tung oil employed 90 may be widely varied, depending, for instance, upon the exact character of the article to be produced, I have had excellent results by using twenty per cent. by weight of tung oil, but this percentage may be increased or diminished very considerably.

95 While I have herein particularly described the manufacture of artificial cork, this novel process may also be used to advantage in the manufacture of other artificial compositions. That is to say, instead of mixing the tung oil with cork particles, I 100 may use tung oil with wood-flour, cellulose, or other fibrous or cellular organic material, and treat the mixture in the manner above described for the treatment of the mixed tung oil and cork.

105 I am, of course, familiar with the fact that tung oil has been used in the linoleum industry in the manufacture of linoleum.

In that industry, however, the oil is first solidified and is then ground and mixed with the cork and other fillers. This is radically different from my present invention, in the practice of which it is necessary that the solidification of the oil shall take place in contact with the particles.

While, as above stated, the exact temperature employed may vary, it should in all cases be below that at which the cork will be injuriously affected, and where the appended claims specify a relatively low temperature, or similar term, they are to be understood in this sense. Also, while the period of heat treatment will vary with the temperature employed and the mass being treated, it is a period much longer in all cases than that usually required for the oxidation of oils by heating, and the term "relatively prolonged period" as used in the claims is to be so understood and meaning a period in excess of twenty-four hours.

I claim:

1. The herein described method of manufacturing artificial cork articles, which consists in mixing pulverized or granulated cork with liquid unoxidized tung oil, and subjecting the material to the action of heat to solidify the oil while in contact with the cork particles; substantially as described.

2. The herein described method of manufacturing artificial cork articles, which consists in mixing pulverized or granulated cork with liquid unoxidized tung oil, then shaping the mixture, and then subjecting the shaped masses to the action of heat to solidify the oil while in contact with the cork particles; substantially as described.

3. The herein described method of manufacturing artificial cork articles, which consists in mixing granulated or pulverized cork with liquid unoxidized tung oil, and then subjecting the mixture to the action of heat at a temperature below that at which the cork will be injured and for a relatively prolonged period to thereby solidify the oil; substantially as described.

4. The herein described method of manufacturing artificial cork articles, which consists in mixing granulated or pulverized

cork with liquid unoxidized tung oil, compressing the mixture into molds, and subjecting the material while in the molds to the action of heat of such temperature and for such period as to effect the solidification of the tung oil without injuring the cork; substantially as described.

5. The herein described method of manufacturing artificial cork, which consists in mixing granulated or pulverized cork with liquid unoxidized tung oil and a suitable solvent, and subjecting the mixture to the action of heat of a relatively low temperature and during a relatively prolonged period to solidify the tung oil without injuring the cork; substantially as described.

6. The herein described method of manufacturing compositions of matter which consists in mixing fibrous or cellular organic material with liquid unoxidized tung oil, and subjecting the mixture to the action of heat at a relatively low temperature and during a relatively prolonged period of time to thereby solidify the oil without injury to the cork; substantially as described.

7. The herein described method of manufacturing artificial cork, which consists in mixing granulated or pulverized cork with not more than forty per cent. of liquid unoxidized tung oil, and subjecting the mixture to the action of heat at a relatively low temperature and during a relatively long period to solidify the tung oil without injuring the cork, substantially as described.

8. The herein described method of manufacturing artificial cork, which consists in mixing granulated or pulverized cork with not more than twenty-five per cent. of liquid unoxidized tung oil, and subjecting the mixture to the action of heat at a relatively low temperature and during a relatively long period to solidify the tung oil without injuring the cork, substantially as described.

In testimony whereof, I have hereunto set my hand.

HERBERT PASCHKE.

Witnesses:

GEO. B. BLEMING,  
GEO. H. PARMELER.